

Patented Dec. 21, 1926.

1,611,799

# UNITED STATES PATENT OFFICE.

MASAAKI YONEZU, OF TOKYO FU, AND EITARO ENDO, OF TOKYO, JAPAN.

## DURABLE PEN.

No Drawing.

Application filed April 23, 1924. Serial No. 708,567.

This invention relates to a pen made with a metal of the iron group, such as nickel, iron or alloy of nickel and iron, containing from 8 to 30% of chromium, and the object 5 thereof is to obtain a pen that endures wear and is not corroded by ink.

An alloy of a metal of the iron group, such as nickel or iron containing a large proportion of chromium, has a characteristic of resisting wear no matter what its hardness is. For instance, if the alloy above described is turned in a lathe, the bit if made of common tool steel of greater hardness will rapidly wear off and become utterly useless very soon. Comparing this with the case in which common carbon steel is turned, there is a marked difference in the life of the bit, which clearly proves this special characteristic of the alloy.

20 This property is most apparent in an alloy of nickel and iron mingled with chromium, but it is also possessed by an alloy of nickel and chromium, or iron and chromium, though a little less in degree.

25 In this invention, advantage is taken of the above property, together with the known corrosion resisting property of high chromium alloys, in making durable pens.

These properties increase in degree ac-

cording to increase of proportion of chromium, but too much chromium makes the manufacture of pens difficult as the alloy becomes less malleable. The proportion of chromium should therefore be limited to from 8 to 30%. In manufacturing pens 30 with this alloy, the addition of a small proportion, as required, of vanadium, manganese, aluminium and other metals will make the manufacture easier and does not decrease in the least the durability of the pens 35 produced.

The normal life of pens made of an alloy of chromium 20%, nickel 5%, and vanadium 4%, the remainder being iron, is twenty times longer than that of steel pens hitherto in use of greater hardness.

We claim:—

1. A writing pen made with an alloy of a metal of the iron group containing 8 to 30% of chromium and 1 to 10% of vanadium.

2. A writing pen made with an alloy of iron and nickel containing 8 to 30% of chromium and 1 to 10% of vanadium.

In testimony whereof we have signed our 55 names to this specification.

MASAAKI YONEZU.  
EITARO ENDO.